

D. E. Hayward,

Shoe Sole,

№ 40,408,

Patented Oct. 27, 1863.

Fig. 1.



Fig. 2.



Fig. 3.



Witnesses,  
John Bowen,  
F. E. Fischmacher.

Inventor,

D. E. Hayward

# UNITED STATES PATENT OFFICE.

DANIEL E. HAYWARD, OF MELROSE, MASSACHUSETTS.

## IMPROVEMENT IN BOOTS AND SHOES.

Specification forming part of Letters Patent No. 40,408, dated October 27, 1863.

*To all whom it may concern:*

Be it known that I, DANIEL EDWIN HAYWARD, of Melrose, in the county of Middlesex and State of Massachusetts, have invented an Improvement in Boots and Shoes, of which the following is a full, clear, and exact description, reference being had to the accompanying drawings, making part of this specification, in which—

Figure 1 is a view of my improved boot; Fig. 2, a view of the sole as seen from beneath; Fig. 3, a section upon the line *x x* of Fig. 1.

Boots and shoes have been made having vulcanized india-rubber soles secured to the inner sole and upper leather by nails which are clinched upon an iron plated last; but soles thus secured are not suitable for certain work—such as ladies' shoes or boots of high cost—as the nails are soon rusted by the moisture of the foot, and are thus liable to discolor the stockings. Where the india-rubber is cemented to the boot it is liable to be torn off, and is easily loosened and detached, if brought near to the fire.

My invention consists in a new article of manufacture—viz., an india-rubber boot or shoe sole having a channel therein for the stitches to lie in, said channel being formed in the sole in the molds in which the sole is vulcanized.

To enable others skilled in the art to understand my invention, I will proceed to describe the manner in which I have carried it out.

My improved sole is made of any suitable rubber compound, and is vulcanized in a mold, within which is arranged a wire which forms the groove *f* in the tread of the sole. This groove has a double object: First, it serves as a guide to the sewing-machine and insures

the placing of the stitches at the proper distance from the edge of the sole; second, it throws the stitches so far beneath the bottom of the sole that the latter may be worn nearly through before the stitches are exposed to wear. The sole thus formed is secured to the boot by sewing upon any machine calculated for sewing the soles of shoes to the uppers, the groove *f*, as before stated, serving as a guide for the machine in placing the stitches.

The compound which I have found to answer the purpose is made as follows: eight pounds crude rubber, two pounds litharge, one pound white lead, one pound lamp-black, four pounds calcined plaster, and six ounces flowers of sulphur. The above compound is then ground upon the ordinary heated rolls, and after being placed in the molds is vulcanized by exposure for ten hours, or thereabout, to a heat of 275° Fahrenheit. I do not, however, confine myself to any particular ingredients, or to any special proportions of the same, nor to any determined degree of heat for vulcanizing the same.

I do not claim a grooved, checkered, or roughened sole of rubber, such as are designed to be nailed onto a boot or shoe; but

What I do claim as a new article of manufacture is—

An india-rubber sole for boots and shoes that is to be sewed thereon, and that has a channel therein for the stitches to lie and be protected in, said channel being formed along the edge of the sole by the molds in which it is formed and vulcanized, substantially as herein described.

D. E. HAYWARD.

Witnesses:

SAM COOPER,  
N. W. STEARNS.